

W. B. SCHULTE.

DRY CELL AND METHOD OF MANUFACTURING THE SAME.

APPLICATION FILED MAY 15, 1920.

1,370,055.

Patented Mar. 1, 1921.

Fig. 1.



Fig. 2.



Inventor

Walter B. Schulte

By his Attorneys

Pennie Davis, Marvin & Edmunds

# UNITED STATES PATENT OFFICE.

WALTER B. SCHULTE, OF MADISON, WISCONSIN, ASSIGNOR TO BURGESS BATTERY COMPANY, A CORPORATION OF WISCONSIN.

## DRY CELL AND METHOD OF MANUFACTURING THE SAME.

1,370,055.

Specification of Letters Patent.

Patented Mar. 1, 1921.

Application filed May 15, 1920. Serial No. 381,653.

To all whom it may concern:

Be it known that I, WALTER B. SCHULTE, a citizen of the United States, residing at Madison, in the county of Dane, State of 5 Wisconsin, have invented certain new and useful Improvements in Dry Cells and Methods of Manufacturing the Same; and I do hereby declare the following to be a full, clear, and exact description of the invention, such as will enable others skilled in the art to which it appertains to make and use the same.

The present invention relates to dry cells and particularly to the cathodes of such 15 cells, and to the method by which the cathodes are provided with a wrapping of bibulous material to prevent the electrode from disintegrating into the electrolyte, particularly during the assembly of the several 20 parts into a complete dry cell.

It is an object of the present invention to eliminate air bubbles within the bibulous envelop or between the envelop and the gelatinized paste commonly used in dry cells 25 of the so-called "bag" type.

It is a further object of the invention to eliminate some of the tedious hand labor incident to the use of a cheesecloth bag or envelop held in place by a wrapping of 30 thread.

Other objects and advantages of the present invention will be made clear by the following detailed description, which is to be taken in conjunction with the accompanying 35 drawings, wherein Figure 1 is a perspective view of a dry cell cathode constructed in accordance with the present invention, and Fig. 2 is a sectional elevation through a complete dry cell.

In the manufacture of dry cells, it is customary to prepare a mixture or "mix" of manganese dioxide, such as pyrolusite, together with carbonaceous material, such as graphite and retort carbon, and usual salts 40 and water, as explained, for instance, in Burgess U.S. Patent No. 1,162,449, dated November 30, 1915, and then to compress this damp and plastic mixture about a carbon rod to form a "core," or cathode, for the dry cell.

50 This molding of the plastic mix into cylin-

drical form with a carbon rod in the center may be done in suitable apparatus, as, for instance, in the tamping machine of Hambuechen U. S. Patent No. 1,232,297, dated July 3, 1917. The cathodes so formed, 55 although strong enough for manipulation on a factory basis, are nevertheless fragile in character and subject to disintegration, particularly if their moisture content is changed substantially from that at which 60 they are molded. As they come from the molding machine, ready for wrapping, they are so soft that it is possible for the operator easily to crush them between his thumb and forefinger.

A customary way of protecting such a molded cathode from disintegration during the further steps in the assembly is to wrap the core with cheesecloth. The cheesecloth ordinarily used is a fine grade, unsized material, and in conformity with usual practice, is held in place around the core with a wrapping of thread. The cloth is brought around the bottom of the core and over the top, and the thread is wound not only 65 around the perimeter of the core, but also longitudinally and parallel with the carbon pencil. The wrapped core so produced can then with advantage be dipped into a very shallow layer of melted paraffin to form an 70 insulating layer or film across the bottom, as explained, for instance, in Burgess U. S. Patent No. 1,211,363, dated January 2, 1917. The cheesecloth is expensive, and the operation of winding the wrapped cores with 75 thread, being a hand operation, is tedious and likewise expensive. Also, there is danger that through unskilled handling, the soft and plastic cores will be deformed. Also some of the active mix may find its 80 way to the outside of the cheesecloth wrapping, and on assembly of the dry cell, be washed over into contact with the zinc, where it can produce local action with 85 destructive results.

In conformity with the method of the present invention, the bibulous envelop or wrapping for the cathode is held in place, not by winding with thread, but by means of an adhesive. This method permits the 90 95 100

use either of paper or of cheesecloth as the bibulous material, and there is some economy in labor. But of more importance than this is the gain in the quality of the 5 dry cell because of the absence of air bubbles within and without the bibulous envelop, as hereinafter explained more at length.

If cheesecloth is to be used as the bibulous 10 envelop, it may be of the quality now commonly used for this purpose. If paper is to be used, as the wrapping, it should be a good quality, thin and porous tissue paper. A slightly calendered surface is not objectionable. The adhesive which I have found 15 the most suitable is one that is thin but does not settle. A starch paste suitable for this work may be made by adding arrowroot to boiling water to the extent of about 20 one per cent. by weight, though other starches and other adhesives can be used. The adhesive should have a sizing property—that is to say, should fill the pores of the paper or of the cheesecloth rather 25 than soak through it, though according to the present method, some soaking through is to be expected because of the relatively large quantity of adhesive which is applied to each of the cores.

30 The procedure for applying the envelop to the core consists in dipping each molded core into the arrowroot solution and then, while the core is still wet from the adhesive, wrapping it with the dry cheesecloth or 35 paper and folding down the wrapping at both ends of the core to cover its top and bottom, care being taken to press out any air bubbles and to secure intimate union between the wrapping and the sticky surface 40 beneath. This operation calls for some skill and judgment. The difficulties are that the core is liable to an incipient breaking up when it is dipped into the adhesive, thereby soiling and impairing the adhesive. Furthermore, the core takes up in its pores an 45 appreciable quantity of the adhesive, thereby becoming softer and more difficult to manipulate during subsequent manufacturing operations. After being wrapped, the 50 cores must be separated from each other in the trays during the time that they are drying, as otherwise they may stick to one another because of the soaking through of some of the adhesive held by the core.

55 There is a tendency, also, for the carbon to loosen from the core just during the time that the paste is setting. These difficulties are not, however, serious, and once appreciated, can be adequately guarded against.

60 After the cores have been wrapped and dried, they can be introduced into their respective zinc cups and a gelatinizable electrolyte can be poured in to fill the space between the zinc and the bibulous envelop.

65 Then, after cooking or such other treatment,

if any, as is necessary to gelatinize the electrolytic paste, the cell can be finished off in usual manner.

The construction above described is illustrated in the drawing, where 1 is the carbon rod with its brass cap 2, and where the molded mix 3 is wrapped about with a sheet of paper 4, a fragment of which, in the drawing, is illustrated as turned and folded down at 5 to diagrammatically illustrate the character of the wrapping. The bottom of the core has a film 6 of paraffin formed by dipping the core into a thin layer of melted paraffin. 7 is the zinc electrode or anode, 8 is the gelatinized paste, 9 is a paraffin paper washer, and 10 is a layer of pitch or sealing wax.

Because of the method by which the envelop is applied to the core, no air bubbles need be entrapped between it and the core. 85 Enough of the adhesive comes out of the pores of the core to fill the pores of the wrapping, and, consequently, after the core has been placed in its zinc cup, and the gelatinizable electrolyte has been introduced, the electrolyte will wet and make good contact with the outer face of the starch-filled envelop, thereby avoiding entrapment of air on the outer face of the envelop. The envelop is of uniform electrical conductivity, and because of the absence of air bubbles, the "flash" of the battery is higher. The process effects a saving 90 both of labor and material, and permits the easy substitution of paper for the more expensive cheesecloth wrapping now commonly used.

It is not readily feasible merely to substitute paper for cheesecloth and wrap it around with thread, for the paper is stiff 105 and tears, and air bubbles are formed within the envelop which give a low flash to the battery and otherwise impair its quality.

In my application Serial No. 381,652, filed concurrently herewith, I have described and 110 claimed broadly a dry cell cathode of the bag type having a bibulous envelop pasted in place, and I have claimed the step which consists in pasting the bibulous envelop to the cathode preparatory to addition of the 115 electrolyte.

I claim:—

1. A dry-cell cathode impregnated in part, at least, with an adhesive, and having a bibulous envelop held in place by said adhesive substantially as described.

2. A dry-cell cathode impregnated in part, at least, with a starch adhesive, and having a bibulous envelop held in place by said adhesive substantially as described.

3. A dry-cell cathode impregnated in part, at least, with a starch adhesive, and having a paper envelop held in place by said adhesive, substantially as described.

4. In the manufacture of dry-cells, the 130

steps which consist in partially impregnating a molded cathode with an adhesive, and then wrapping said cathode with a bibulous envelop and thus securing said envelop in place, substantially as described.

5. In the manufacture of dry-cells, the steps which consist in partially impregnating the molded cathode with a starch adhesive, and then wrapping said cathode with

a paper envelop and thus securing said envelop in place, substantially as described.

6. In the manufacture of dry-cells, the steps which consist in dipping the molded cathode in a suitable adhesive, and then wrapping said cathode in paper, substantially as described.

In testimony whereof I affix my signature.  
WALTER B. SCHULTE.